

Dec. 18, 1934.

H. P. HAYDEN

1,985,092

METHOD OF PRODUCING CONCRETE STRUCTURES

Filed March 5, 1929



FIG. 1.



FIG. 2.



FIG. 3.

INVENTOR

WITNESS:

John P. Kitchell.

Harold P. Hayden

BY

Brown & Harding.

ATTORNEY.

## UNITED STATES PATENT OFFICE

1,985,092

METHOD OF PRODUCING CONCRETE  
STRUCTURESHarold P. Hayden, Woodbridge, N. J., assignor to  
The Barber Asphalt Company, Philadelphia,  
Pa., a corporation of West Virginia

Application March 5, 1929, Serial No. 344,597

1 Claim. (Cl. 18—47)

My invention relates to method of producing concrete structures and more particularly relates to concrete structures of the type which are produced by the pouring of concrete into forms.

Heretofore for the production of concrete structures such, for example, as are produced by pouring concrete into forms, the forms being removed after the concrete has set or reached a condition of required rigidity, substantial difficulty has been met with in effecting proper curing of the concrete and the structures produced have been subjected to internal stresses and strains due to changes in the moisture content of the structure. Changes in temperature also result in the development of certain types of stresses in concrete structures due to the expansion or contraction of an element in the structure resulting from such change in temperature. Allowance for the anticipated variation of dimensions due to temperature changes is made in the design of the structure, usually by the provision of expansion joints and variations in the dimensions of concrete structures due to changes in the moisture content thereof may be taken care of similarly. However, in concrete structures, and more particularly where, for example, the concrete structure is reinforced with steel or the like, internal stresses develop within the structure as a result of change in dimensions of the structure resulting from variations in the moisture content thereof and which cannot be taken care of as can change in dimensions as such.

Heretofore the curing of concrete forming structures of the character produced by the pouring of concrete into forms has been more or less adequately accomplished by permitting the forms to remain on the structure throughout the duration of the stipulated curing period, or at least until the structure is sufficiently rigid to permit the removal of the forms. However, where wooden forms are used, even though permitted to remain in place until the concrete is cured, much of the water necessary to complete the hydration of the Portland cement is lost by evaporation through the porous form wall unless the forms are frequently wetted during the curing period and in cases where the forms are removed prior to the end of the stipulated curing period, it has been necessary to frequently wet the exposed surface of the structure in an effort to maintain a sufficient amount of water in the concrete to effect the hydration of the Portland cement.

As a result of my investigations, I have discovered that it is possible to produce concrete

structures of the character produced by the pouring of concrete into forms which have increased strength and which will be free from the internal stresses incident to variations in the moisture content thereof throughout the life of the structure, by the encasement of the structure in a water impervious system at the time of pouring the concrete into the form. It will be apparent that it is unnecessary to make provision for dimensional changes in the concrete structure due to changes in the moisture content thereof in structures so encased, as such dimensional changes will be obviated.

Now, it is the object of my invention to provide a method of producing concrete structures, such as are produced by the pouring of concrete into forms, by which the mixing water will be conserved within the structure for the complete hydration of the cement and the moisture content of the structure after the completion of such hydration will be permanently stabilized with the result that a structure of maximum strength may be developed which will be free from the stresses which would result from changes in the moisture content thereof.

In accordance with my invention I provide a method for the application of a water impervious film to the concrete as it is poured into the forms, the film acting to insure the retention in the body of the concrete of initial moisture sufficient for hydration of the cement content with maximum efficiency. At the same time my method contemplates provision for the retention of the film on the concrete structure on removal of the forms, the film as originally applied, or as it may be supplemented, acting, after removal of the forms, to maintain the moisture content of the concrete at a substantially constant percentage regardless of variations in atmospheric conditions or other conditions which would tend to influence the moisture content thereof.

In the adaptation of the method in accordance with my invention to practice from the broad standpoint, I provide the forms, into which the concrete is to be poured, with a coating of a material capable of supporting the water impervious film to be applied to the concrete. The coating serves to support the film of water impervious material during the pouring of the concrete into the forms and is of such a character that after the concrete has been poured and desirably puddled, the adherence of the film to the concrete will be greater than its adherence to the coating material, or than the adherence of the coating material to the forms, with the result

that on removal of the forms the water impervious film will remain adhered to the concrete. After removal of the forms any coating material adhering to the film is removed and if desired the film 5 may be supplemented.

It will be understood that from the broad standpoint my invention contemplates the application of a water impervious film to concrete as it is poured into forms and the retention of the film 10 by the concrete after the forms are removed, the application of the film being effected through the medium of a film supporting coating initially applied to the forms.

In carrying the method in accordance with my 15 invention into practice, any type of forms for the formation of concrete structures may be used. However, the carrying out of the method will be facilitated where forms of the type which comprise sections composed of back and sides built 20 in place and having a separable front section adapted to be secured in place when the concrete is to be poured, are used. As an illustration of the practical adaptation of the method in accordance with my invention in, for example, the 25 construction of a wall, the forms, for example, of the type having back and sides built in place and a removable front, having been constructed, the interior of the forms, including the separable front section if the form is of such type, 30 are coated with a coating of, for example, clay slurry, white wash, or the like, the application being made, for example, by brushing or by a spray gun, and there is formed upon the coating a water impervious film, for example, formed of a linseed oil paint, rubber latex, bitumen or bituminous material as, for example, asphalt, or of coal tar pitch, or the like. The water impervious film may be formed upon the coating, 35 for example, by brushing or spraying upon the coating a water external phase bituminous emulsion, heated asphaltum, or asphaltum dissolved or cut back by means of a suitable solvent. Where the water impervious film is formed through the use of heated asphalt, or asphalt solution, the 40 clay slurry coating should be permitted to dry before application of the film forming material. However, where the film is formed by the use of a bituminous emulsion, drying of the clay slurry coating is not necessary prior to applica- 45 tion of the film.

After the formation of the water impervious film, as described above, the concrete is poured into the form and the surface thereof, at the 50 open top of the form, coated directly with a material which will form a water impervious film, for example, a material similar to that used in forming the water impervious film on the coated forms as, for example, a bituminous emulsion or an asphalt solution, heated asphalt, coal tar pitch, or the like. The concrete is then permitted to set and when it has set or hardened 55 sufficiently, the forms are removed. On removal of the forms the water impervious film will remain adhered to the concrete, since the adherence of the film to the concrete, as will be hereinafter described, may be made greater than to the clay coating; in any event the adherence of the water impervious film to the concrete will be greater than the adherence of the clay coating to the forms so that on removal of the forms the film will remain with the concrete structure 60 formed. If desired, and more especially where the water impervious film is formed with heated asphalt or asphalt solution, the adherence of the film to the concrete may be insured by the addi-

tion to the film after its formation and before it has set of a sharp mineral aggregate, as relatively finely crushed stone, slate, or the like, which will provide the film with a tooth for engagement with the concrete.

After the forms are removed from the concrete, if it be that the water impervious film adhering to the structure carries with it, in whole or in part, the coating initially applied to the forms as a basis for the formation of the film, the coating is removed as, for example, by washing it off, and the water impervious film, if it were damaged, for example, by the tools used in puddling the concrete, is repaired with material of the same character as that used in forming the film, in order to insure the envelopment of the surfaces of the concrete structure by the water impervious film. Alternatively, after removal of the forms and any of the material used for initially coating the forms, the film may be simultaneously repaired and supplemented by the application to the concrete structure of a coating of, for example, hot asphalt, asphalt solution, or asphalt emulsion, by means of brushing or through the use of a spray gun. The film may be supplemented by a coating of any desired weight and may be supplemented by more than one coating if desired. Under circumstances where the concrete structure is so placed as to be subjected to the direct action of the elements, the initial film 30 may be supplemented by the application of weather resistant material, as for example, by the application of bituminously impregnated fabric, for example, such as asphalt impregnated felt, the application of which may be effected, for example, by first coating the film with a mopping of hot asphalt, or of asphalt solution, or the like, then applying the saturated fabric in sheet form while the asphalt coating is in an adhesive condition and finally coating the fabric and sealing 35 the joints between the strips thereof with, for example, heated asphalt or asphalt solution. It may also be desirable to embed a granular aggregate such as slag, crushed stone or slate in the surface of the supplementary coating in order 40 that a layer of Portland cement or magnesite stucco, or the like, may be adhered thereto for the purpose of more permanently protecting the surface of the structure and also for the purpose of 45 decoration thereof.

While it will be understood that the method embodying my invention may be carried out without the use of any special apparatus, I have illustrated in the accompanying drawing the application of the method embodying my invention to the production of a concrete block.

In the accompanying drawing:

Fig. 1 is a sectional view of a mould composed of form members ready for the reception of a charge of concrete.

Fig. 2 is a sectional view of the mould shown in Figure 1, the concrete having been poured.

Fig. 3 is a perspective view, partly broken away, showing a block produced in the mould of Figures 1 and 2, the form members removed from the block being indicated.

In the several figures *a* indicates form members, comprising in the present case sides and ends arranged together to form a mould for the production of a block. *b* indicates a coating of, for example, clay slurry applied to the interior surface of the members forming the mould and *c* indicates a coating of bituminous material, as asphalt applied over the coating of clay slurry. *d* indicates a mass of concrete poured into the

5 mould, while c' indicates a coating or film of asphalt applied over the surface of the concrete after pouring into the mould. e indicates the finished concrete block, the form members a composing the mould having been removed. The block, it will be noted, is entirely encased with asphalt due to adherence to it of the asphalt coating c applied interiorly of the mould and the asphalt coating c' applied to the top of the concrete after pouring into the mould. The asphalt coating c is prevented from adhering to the interior of the mould rather than to the outside of the block owing to the coat of clay slurry which is applied directly to the mould and which, as 10 shown in Figure 3, remains on the form members 15 on their removal from the block.

It will now be observed that as a result of my invention provision is made for the application 20 to concrete as it is poured into forms of a water impervious film, which coats the entire surface 25 of the concrete and which serves to prevent evaporation of water from the concrete after pouring and during the curing period, when the maintenance of requisite water is essential to the sufficient hydration of the cement content for 30 adequate curing and, at the same time, provision is made for insuring the retention of the film by the concrete structure after the removal of the forms with the result that the moisture content 35 of the concrete will be stabilized during the life of the concrete structure by the fact that the water impervious film will protect the body of the concrete from the effect of variations in the moisture content of the atmosphere or other variable conditions which would tend to affect the moisture content of the concrete structure. As has been described, the film may be supplemented to a greater or less degree after the removal of the

forms where conditions or service of the concrete structure are such as to require a protective coating of greater durability than that afforded by the initial film which is desirably of no very great thickness, though it will be appreciated that it may be made initially of any desired thickness within reasonable limits.

As a result of my invention, concrete structures such as are produced by the pouring of concrete into moulds or forms may be produced with maximum initial strength and free from internal stresses and strains arising from variations in the moisture content thereof through change in the moisture content of contiguous bodies or atmospheric humidity.

It will be understood that I do not intend that my invention shall be limited to the precise procedure described herein by way of illustration, nor to the use of any particular material for the formation of the water impervious film or for supplementing it, the use of any material capable of producing the results herein described being contemplated by me, though the method will be economically and effectively carried out through the use of bituminous material, as for example, asphaltum, which may be used, as has been indicated, in a heated condition, in solution in a suitable solvent, or, and which is perhaps preferable, in the form of an emulsion.

Having now fully described my invention, what 30 I claim and desire to protect by Letters Patent is:

A parting medium adapted for the coating of a mold for concrete and for the support of a flexible, water-impervious film to be adhered to concrete formed in the mold, comprising a coating of 35 clay formed by the application of an aqueous clay slurry to the mold.

HAROLD P. HAYDEN.